

[72] Inventors **Haruo Ishida**  
Hirakata-shi;  
Kiyoshi Otaka, Hyogo-ken, both of Japan  
[21] Appl. No. **787,237**  
[22] Filed **Dec. 26, 1968**  
[45] Patented **Nov. 23, 1971**  
[73] Assignee **Daiwa Chemical Industries Ltd.**  
Osaka-shi, Japan  
[32] Priority **Dec. 29, 1967**  
[33] **Japan**  
[31] **42/84829**

[54] **PROCESS FOR MANUFACTURING BULKY  
FABRICS**  
2 Claims, No Drawings

[52] U.S. Cl. .... **117/62,**  
117/139.5 CE  
[51] Int. Cl. .... **B44d 1/44**  
[50] Field of Search. .... **117/62,**  
139.5 I, 63, 139.4; 28/76, 74; 8/130.1

[56] **References Cited**  
UNITED STATES PATENTS  
758,311 4/1904 Goldman..... 106/150  
Primary Examiner—William D. Martin  
Assistant Examiner—M. Sofocleous  
Attorney—Larson, Taylor and Hinds

**ABSTRACT:** A process for producing a bulky fabric which comprises impregnating a fabric with a bound water-containing metal salt, heating the impregnated fabric to expand said metal salt contained in the fabric, heat-setting the resultant fabric and washing with water the resultant fabric to remove the expanded metal salt; said bound water-containing metal salt being expandable by the emission of its own bound water when heated at a temperature of from 100° C. to a second order transition temperature of the fiber to produce the expanded metal salt soluble in water but not melting or decomposing at a temperature applied in said heat-setting step.

**PROCESS FOR MANUFACTURING BULKY FABRICS**

This invention relates to bulky fabrics such as bulky woven and knitted fabrics and the manufacture thereof. More particularly, the invention pertains to a novel process for manufacturing bulky fabrics and a novel intermediate fabrics for preparing bulky fabrics.

In general, bulky fabrics are prepared in the prior art by weaving bulky yarns into a textile fabric and heat-setting it. In the heat-setting process temperatures higher than second order transition temperature of the fibers constituting the fabric are usually applied to heat-set the fabric. When fabrics of synthetic fibers which are heat-shrinkable are heated at such high temperatures, however, undesirable shrinkage of the fabrics occurs to the extreme degree, making it difficult to produce fabrics having excellent bulkiness, softness, hand and the like characteristics. While lengthwise and widthwise shrinkage of the fabric can be prevented to some extent by using a tenter or other mechanical means, it is inevitable that the extreme shrinkage occurs in thickness of the fabric, reducing the thickness of the fabric and resulting in the product hard to the touch.

Further, the creases produced in the fabric during dyeing and finishing steps have so far been removed by ironing, pressing or tentering, but in such a case some shrinkage of the fibers is unavoidable. To prevent the creation of the creases dyeing and finishing of bulky fabrics have been done in the prior art using special machines such as beam dyeing machine, jet dyeing machine, open-soaper, etc., but the equipment as above calls for enormous expenditure for installation and operation.

An object of the invention is to provide bulky fabrics having excellent bulkiness, softness, hand, shrink-proof property, crease-proof property, pleating property and draping property.

Another object of the invention is to provide a process for manufacturing bulky fabrics having above characteristics free from the drawbacks of the conventional processes.

A further object of the invention is to provide expanded fabrics resistant to heat applied in the heat-setting step and capable of producing bulky fabrics having above characteristics free from undesired shrinkage.

The above and other objects and advantages of the invention will be apparent from the following description.

According to the researches of the present inventors, it has been found that when a woven or knitted fabric is impregnated with a certain kind of bound water-containing metal salts and heated at a temperature not lower than 100°C. to expand the metal salts, a unique expanded fabric containing expanded metal salts interposed in the intervals between fibers of the fabric can be obtained and that when such an expanded fabric is subjected to a heat-setting step, such fabric is set in the expanded form without showing any shrinkage and a bulky fabric having excellent properties is produced after the removal of the expanded metal salts contained therein.

The fabrics used in the invention include woven fabrics and knitted fabrics prepared from at least one of synthetic fibers which are heat-shrinkable. Examples of the synthetic fibers are polyester, polyamide, polyacrylonitrile, polyurethane, polyvinyl chloride, polypropylene and the like fibers. Further, the fabrics made of mixed yarn of said synthetic fibers and natural or semisynthetic fibers, and the fabrics in which the yarn of said synthetic fibers and that of natural or semisynthetic fibers are combined can also be used in the invention.

The bound water-containing metal salts used in the invention should have properties expandable by the emission of their own bound water when heated at a temperature of from 100°C. to below a second order transition temperature of the fibers constituting the fabric to produce the expanded metal salt soluble in water but not melting or decomposing at an elevated temperature applied in the heat-setting step, i.e., a temperature of a second order transition temperature to below a decomposing temperature of the fibers. In the invention various metal salts having above properties can be used, which include organic metal salts, inorganic metal salts, dou-

ble salts and complex salts. Typical examples of such metal salts are hydrous calcium chloride ( $\text{CaCl}_2 \cdot 2\text{H}_2\text{O}$  or  $\text{CaCl}_2 \cdot 6\text{H}_2\text{O}$ ), hydrous sodium tetraborate ( $\text{Na}_2\text{B}_4\text{O}_7 \cdot 10\text{H}_2\text{O}$ ), hydrous sodium acetate ( $\text{CH}_3\text{COONa} \cdot 3\text{H}_2\text{O}$ ), hydrous aluminum sulfate [ $\text{Al}_2(\text{SO}_4)_3 \cdot 18\text{H}_2\text{O}$ ], hydrous aluminum potassium sulfate [ $\text{KA}_1(\text{SO}_4)_2 \cdot 12\text{H}_2\text{O}$ ], hydrous magnesium chloride ( $\text{MgCl}_2 \cdot 6\text{H}_2\text{O}$ ), hydrous sodium potassium tartrate ( $\text{KNaC}_4\text{H}_4\text{O}_6 \cdot 4\text{H}_2\text{O}$ ), hydrous sodium thiosulfate ( $\text{Na}_2\text{S}_2\text{O}_3 \cdot 5\text{H}_2\text{O}$ ), hydrous sodium silicate ( $\text{Na}_2\text{O} \cdot x\text{SiO}_2 \cdot y\text{H}_2\text{O}$ ), hydrous sodium metasilicate ( $\text{Na}_2\text{SiO}_3 \cdot 5\text{H}_2\text{O}$ ), etc.

When these metal salts are heated at a temperature of higher than 100°C., they are first dissolved in their own bound water and emit the water in a gaseous state to produce 15 micelike expanded solids of the metal salts which are soluble in water but can not be melted nor decomposed at an elevated temperature to be applied in the setting step of the fabric. The expanded volume of the metal salts may vary depending on the kind of the metal salts used and the heat conditions to 20 decompose the metal salts. Preferable heat conditions are represented in the Table 1 below, in which expanded volume is determined by the following equation.

$$25 \text{ Expanded volume (\%)} = \frac{\text{Volume of metal salt expanded}}{\text{Volume of bound water-containing metal salt used}} \times 100$$

TABLE I

|    | Formula of metal salt                                               | Preferable Blowing Temperature (°C.) | Expanded Volume (%) |
|----|---------------------------------------------------------------------|--------------------------------------|---------------------|
| 35 | $\text{CaCl}_2 \cdot 2\text{H}_2\text{O}$                           | 100-130                              | 170                 |
|    | $\text{CaCl}_2 \cdot \text{H}_2\text{O}$                            | 100-130                              | 140                 |
|    | $\text{Na}_2\text{B}_4\text{O}_7 \cdot 10\text{H}_2\text{O}$        | 100-130                              | 270                 |
|    | $\text{CH}_3\text{COONa} \cdot 3\text{H}_2\text{O}$                 | 100-120                              | 300                 |
| 40 | $\text{Al}_2(\text{SO}_4)_3 \cdot 18\text{H}_2\text{O}$             | 100-150                              | 160                 |
|    | $\text{KA}_1(\text{SO}_4)_2 \cdot 12\text{H}_2\text{O}$             | 100-110                              | 210                 |
|    | $\text{MgCl}_2 \cdot \text{H}_2\text{O}$                            | 100-140                              | 130                 |
|    | $\text{KNaC}_4\text{H}_4\text{O}_6 \cdot 4\text{H}_2\text{O}$       | 100-140                              | 280                 |
|    | $\text{Na}_2\text{S}_2\text{O}_3 \cdot 5\text{H}_2\text{O}$         | 100-130                              | 130                 |
|    | $\text{Na}_2\text{O} \cdot x\text{SiO}_2 \cdot y\text{H}_2\text{O}$ | 100-140                              | 460                 |
| 45 | $\text{Na}_2\text{SiO}_3 \cdot 5\text{H}_2\text{O}$                 | 100-140                              | 470                 |

The metal salts can be used alone or in mixture and in the form of solution, suspension, paste or powder, and various additives may be added thereto, as required. For example, to adjust the blowing temperature, expanded volume and mechanical strength of the expanded solids, there may be added the conventional blowing agents which will emit carbon dioxide gas, ammonium gas, nitrogen gas, etc., by the decomposition thereof when heated. For the same purposes as above fillers, such as metal salts containing no bound water, clay, bentonite, etc., may be added. To improve the stability of the resultant foam surface active agents or starch paste may be added thereto. Further, dyestuffs may also be added to make it possible to dye the fabric simultaneously.

According to the invention fabrics are first impregnated with the metal salts by various means according to the forms of metal salts used, for example, by dipping, padding, coating, spraying, printing, sprinkling, etc. To obtain bulky fabrics having uniform bulkiness throughout the fabric the entire part of the fabrics may be uniformly impregnated with the metal salts, while to obtain bulky fabrics having bulky spots and other bulky patterns the fabrics may be partly impregnated with the metal salts in accordance with the patterns desired. The amount of the metal salts infused into the fabric may be in the range of 2 to 200 weight percent, preferably 20 to 60 weight percent, based on the weight of the fabric. Throughout the specification and claims the expression "weight of the fabric" is intended to mean the weight of the fibers constituting the impregnated part of the fabric. Lesser amount of the im-

pregnation results in poorer effect and higher amount brings no increase in the effect, rendering the process uneconomical. The bulkiness of the final bulky fabric may vary depending on the amount of the impregnation, so that by suitably selecting such amount the bulky fabric having desired bulkiness is obtainable.

The fabrics thus impregnated with metal salts are then subjected to heating step to expand the metal salt after squeezing and/or drying, as required. When dyestuff is used in combination with the metal salts it is preferable to dry the impregnated fabric prior to the heating step to prevent the migration of the dye. The heating step for expanding the metal salts is carried out at a temperature not lower than 100° C. but below second order transition temperatures of the fibers constituting the fabric. Preferable temperatures to be applied may vary in accordance with the kind of the metal salts and fabrics used, and temperatures preferable for the respective metal salts are shown in the foregoing table 1. The time required for the expansion of the metal salts may vary depending in the temperature applied and metal salts used, but usually a period of 0.1 to 10 minutes is sufficient for the purpose.

The resultant fabric contains expanded metal salts interposed in the intervals between fibers of the fabric and easily soluble in water but not melting or decomposing by the heat applied in the subsequent heat-setting process. By the presence of the expanded metal salts the fabric thus obtained is in expanded form. In more detail the respective fibers constituting the fabric are elongated irregularly by the expansion of the metal salts and locked in such conditions by the expanded metal salts. Accordingly, when the expanded fabric is heated at a temperature higher than a second order transition temperature of the fibers the fabric is heat-set without the shrinkage of the fibers locked with the expanded metal salts. The amount of the expanded metal salts interposed in the fabric may be in the range of 1 to 100 weight percent, preferably 10 to 30 weight percent, based on the weight of the fabric.

The bulky fabrics of the invention are prepared by heat-setting the expanded fabric and washing the heat-set fabric with water to remove the expanded metal salts therefrom. The heat-setting treatment is carried out in the conventional manner, for example, by heating the expanded fabric at temperatures of second order transition temperatures to below decomposing temperatures of the fibers constituting the fabric. The preferable temperatures may vary in accordance with the kind of the fibers, but temperatures of not higher than 50° C. above the second order transition temperature of the fibers may usually be applied. The time required for the heat-setting is usually 0.1 to 10 minutes. In this step the fabric shows no shrinkage as the fibers are locked with expanded metal salts.

The fabric thus heat-set is washed with water to remove the expanded metal salts, whereby the bulky fabric having excellent bulkiness, softness, hand, shrink-proof property, crease-proof property, pleating property and draping property is obtained.

In the preferred embodiment of the process of the invention, the heating step for expanding metal salts and heat-setting step are carried out in a single heating apparatus, such as air oven and the like. For example, the fabric impregnated with metal salts is introduced into an air oven through which air heated at a temperature of higher than a second order transition temperature of the fibers is passed. At the initial stage, while the fabric has not been heated yet to a second order transition temperature or higher, the metal salts have expanded, and when the temperature of the fabric reaches the second transition temperature or higher, the fabric is heat-set. In a continuous manner the fabric impregnated with the metal salts is continuously passed through the air oven, and at the inlet portion of the oven the metal salts are expanded, and then the fabric is heat-set.

For better understanding of the invention examples are given below in which all parts are in parts by weight.

## EXAMPLE 1

A woven fabric of polyester yarn in which creases occurred during carrier dyeing process using a dispersed dye was immersed in the following composition and squeezed with a mangle to 80 weight percent impregnation with the composition, based on the weight of the fabric.

|    |                                                                                                                         |                         |
|----|-------------------------------------------------------------------------------------------------------------------------|-------------------------|
| 10 | "Keiso No. 3"<br>(Hydrous sodium silicate<br>containing 60 weight percent<br>of water, specified in<br>JIS K-1408 1966) | 50 parts                |
| 15 | Polyethyleneglycol<br>nonylphenyl ether<br>Water                                                                        | 0.5 parts<br>49.5 parts |

Then the fabric was tentered on a frame with pins to accurate lengthwise and widthwise measurements and placed in an air oven heated at 180° C. for 3 minutes. In the first one minute the sodium silicate expanded, generating water vapor and in the last two minutes the fabric was heat-set. Thereafter the fabric was washed with water to remove the expanded metal salts and dried at 80° C. Thus the bulky fabric having the properties shown in table 2 below was obtained.

For comparison, the same treatment was performed using the composition same as above but not containing hydrous sodium silicate. The results are shown in Table 2 below.

TABLE 2

|    | Changes in hand                                           | Changes in thickness                       | Creases                                                               |
|----|-----------------------------------------------------------|--------------------------------------------|-----------------------------------------------------------------------|
| 30 | Fabric finished according to the method of the invention. | Softness and hand improved.                | Nil..... Completely removed.                                          |
| 35 | Comparative fabric.                                       | Hand hardened and feature of drapery lost. | Decrease of 30%. Originally creased portions remained as depressions. |

## EXAMPLE 2

A woven fabric of polyamide yarn was impregnated with the following composition in the order of 50 weight percent impregnation and dried at room temperature.

|    |                                                                                             |                                  |
|----|---------------------------------------------------------------------------------------------|----------------------------------|
| 50 | Hydrous aluminum potassium sulfate<br>Bentonite (water content: 80 weight percent)<br>Water | 40 parts<br>10 parts<br>50 parts |
|----|---------------------------------------------------------------------------------------------|----------------------------------|

The fabric thus treated was folded into two after inserting pleating paper and placed in an air oven heated at 130° C. for 10 minutes. In the first 3 minutes the aluminum potassium sulfate expanded, generating water vapor and in the last 7 minutes the fabric was heat-set. The removal of the expanded metal salts by washing with water gave the bulky fabric having the properties shown in table 3 below.

For comparison the same treatment was performed using the above composition but not containing hydrous potassium aluminum sulfate. The results are shown in table 3 below.

TABLE 3

|    | Changes in hand                             | Changes in thickness               | Pleat                                                     |
|----|---------------------------------------------|------------------------------------|-----------------------------------------------------------|
| 70 | Fabric finished by method of the invention. | Softness and hand improved.        | Nil..... Excellent pleats.                                |
| 75 | Comparison.....                             | Hand hardened.... Decrease of 40%. | Pleated portions thinned and sharpened and partly shrunk. |

## EXAMPLE 3

A woven fabric of bulky polyester yarn was immersed in the following composition, squeezed with a mangle to 80 weight percent impregnation and dried at 60°C.

|                                        |            |
|----------------------------------------|------------|
| "Foron Blue BL"                        |            |
| (Trade Mark, Sandoz Ltd., Switzerland) | 4 parts    |
| Hydrous potassium tartarate            | 30 parts   |
| Carboxymethyl cellulose                | 1 parts    |
| Sodium metanitrotoluene sulfonate      | 1 parts    |
| Polyethyleneglycol nonylphenyl ether   | 0.5 parts  |
| Water                                  | 63.5 parts |

The fabric thus treated was tentered on a frame with pins and placed in an air oven heated at 180°C. for 5 minutes. In the first 1.5 minutes the hydrous sodium potassium tartarate expanded, generating water vapor and in the last 3.5 minutes the fabric was heat-set. The removal of the expanded metal salts by washing with water gave the bulky fabric having the properties shown in table 4 below.

For comparison the same treatment was performed using the same composition as above but not containing hydrous sodium potassium tartarate. The results are shown in table 4 below.

TABLE 4

| Sample treated according to the method of invention. | Changes in hand | Dyeing property                                                  | Changes in thickness |
|------------------------------------------------------|-----------------|------------------------------------------------------------------|----------------------|
| Softness and hand improved.                          | Excellent       | Nil.                                                             |                      |
| Comparison                                           | Hand hardened.  | Excellent. Slightly darker in colour due to shrinkage of fibers. | Decrease of 32%.     |

## EXAMPLE 4

A textile fabric of high-bulky polyacrylonitrile yarn, in which creases were created during dyeing process was immersed in the following composition, squeezed with a mangle to 80 weight percent impregnation and dried at 60°C.

|                        |            |
|------------------------|------------|
| Hydrous sodium acetate | 30 parts   |
| Hydrous sodium formate | 10 parts   |
| Polyethyleneglycol     |            |
| nonylphenyl ether      | 0.5 parts  |
| Water                  | 49.5 parts |

The fabric thus treated was tentered on a frame with pins and placed in an air oven heated at 130°C. for 2 minutes. In the first one minute the metal salts expanded, generating water vapor and in the last one minute the fabric was heat-set. The removal of the expanded metal salts by washing with water gave the bulky fabric having the properties shown in table 5 below.

For comparison the same treatment was performed using the same composition but not containing hydrous sodium acetate and hydrous sodium formate. The results are shown in table 5 below.

TABLE 5

| Sample finished according to the method of the invention. | Change in hand                                  | Changes in thickness | Crease                                               |
|-----------------------------------------------------------|-------------------------------------------------|----------------------|------------------------------------------------------|
| Softness and hand improved.                               | Nil.                                            | Completely removed.  |                                                      |
| Comparison                                                | Hand hardened and feature of drapery decreased. | Decrease of 35%.     | Originally creased portions remained as depressions. |

## EXAMPLE 5

A textile fabric of polyester yarn in which creases occurred during dyeing step was immersed in the following composition and squeezed with a mangle to 100 weight percent impregnation.

|                            |            |
|----------------------------|------------|
| Hydrous aluminum sulfate   | 25 parts   |
| Hydrous sodium thiosulfate | 25 parts   |
| Polyethyleneglycol         |            |
| nonylphenyl ether          | 0.5 parts  |
| Water                      | 49.5 parts |

The fabric thus treated was tentered on a frame with pins and placed in an air oven heated at 180°C. for 3 minutes. In the first one minute the metal salts expanded, generating water vapor and in the last two minutes the fabric was heat-set. The removal of the expanded metal salts gave the bulky fabric having the properties shown in table 6 below.

For comparison, the same treatment was performed using the same composition as above but not containing hydrous aluminum sulfate and hydrous sodium thiosulfate. The results are shown in table 6 below.

TABLE 6

| 30         | Bulky fabric of the invention. | Change in hand | Change in thickness | Creases                                              |
|------------|--------------------------------|----------------|---------------------|------------------------------------------------------|
| Comparison | Softness and hand improved.    | Hand hardened. | Decrease of 20%.    | Originally creased portions remained as depressions. |

## EXAMPLE 6

Hydrous sodium metasilicate powder was uniformly sprinkled on a woven fabric of bulky polyester yarn in the order of 40 weight percent based on the weight of the fabric and placed in an air oven heated at 180°C. for 5 minutes.

In the first 1.5 minutes the hydrous sodium metasilicate was melted, infused into the fabric and then expanded, generating water vapor, and in the last 3.5 minutes the fabric was heat-set.

Thereafter the fabric was washed with water to remove the expanded metal salts and dried, whereby the bulky fabric soft to the touch was obtained.

## EXAMPLE 7

A woven fabric of polyester fiber dyed by carrier dyeing was immersed in the following composition prior to heat-treatment for removing carrier, squeezed to 80 weight percent impregnation and dried at 100°C.

|                            |            |
|----------------------------|------------|
| Hydrous calcium chloride   | 30 parts   |
| Hydrous magnesium chloride | 20 parts   |
| Polyethyleneglycol         |            |
| nonylphenyl ether          | 0.5 parts  |
| Water                      | 49.5 parts |

The fabric thus treated was placed in an air oven heated at 180°C. for 3 minutes. In the first one minute the hydrous calcium chloride and hydrous magnesium chloride expanded, generating water vapor and in the last two minutes the fabric was heat-set. The fabric was then washed with water to remove the expanded metal salts and dried at 60°C. Thus, the bulky fabric having the following properties shown in table 7 was obtained.

For comparison, the same treatment was performed using the same composition as above but not containing hydrous

calcium chloride and hydrous magnesium chloride. The results are shown in table 7 below.

hydrous sodium potassium tartrate, hydrous sodium thiosulfate, hydrous sodium silicate and hydrous sodium

TABLE 7

|                          | Changes in hand             | Changes in thickness | Creases                                              | Removal of carriers         |
|--------------------------|-----------------------------|----------------------|------------------------------------------------------|-----------------------------|
| Fabric of the invention. | Softness and hand improved. | Nil.....             | Nil.....                                             | Carrier completely removed. |
| Comparison.....          | Hand hardened.              | Decrease of 25%.     | Originally creased portions remained as depressions. | Carrier slightly remaining. |

## EXAMPLE 8

A woven fabric of polyester yarn was immersed in the following composition, squeezed to 70 weight percent impregnation and dried at 80° C.

|                            |            |
|----------------------------|------------|
| Hydrous sodium tetraborate | 40 parts   |
| Polyethyleneglycol         |            |
| nonylphenyl ether          | 0.5 parts  |
| Starch                     | 8 parts    |
| Water                      | 51.5 parts |

The fabric thus treated was tentered on a frame with pins and placed in an air oven heated at 180° C. for 3 minutes. In the first 1 minute the hydrous sodium tetraborate expanded, generating water vapor and in the last 2 minutes the fabric was heat-set. The fabric was then washed with water to remove the expanded metal salts and dried at 80° C. Thus, the bulky fabric soft to the touch was obtained.

What we claim is:

1. A process for manufacturing a bulky fabric which comprises impregnating a synthetic heat shrinkable fabric with 20 to 60 weight percent, based on the weight of the fabric, of a bound water-containing metal salt, said metal salt being at least one species selected from the group consisting of hydrous calcium chloride, hydrous sodium tetraborate, hydrous sodium acetate, hydrous aluminum sulfate, hydrous aluminum potassium sulfate, hydrous magnesium chloride,

- 15 metasilicate, heating the impregnated fabric to a temperature of from 100° C. to below a second order transition temperature of the fibers constituting the fabric to expand said metal salt contained in the fabric, heat-setting the resultant fabric at a temperature ranging from a second order transition temperature to below a decomposing temperature of the fibers and washing with water the resultant fabric to remove the expanded metal salt; said bound water-containing metal salt being first dissolved in its own bound water and emitting the water in a gaseous state when heated at a temperature of from 20 100° C. to a second order transition temperature of the fibers to produce pumicelike expanded solid of the metal salt soluble in water but not melting or decomposing at a temperature applied in said heat-setting step.
- 25 2. An expanded synthetic fabric resistant to heat-shrinkage for producing a bulky fabric which comprises a fabric and 10 to 30 weight percent, based on the weight of the fabric, of expanded metal salts interposed in the intervals between fibers of the fabric and water-soluble but not melting or decomposing 30 at a temperature of between a second transition temperature and below a decomposing temperature of the fabrics, said metal salts being at least one species selected from the group consisting of calcium chloride, sodium tetraborate, sodium acetate, aluminum sulfate, aluminum potassium sulfate, magnesium chloride, sodium potassium tartrate, sodium thiosulfate, sodium silicate and sodium metasilicate.

\* \* \* \* \*

45

50

55

60

65

70

75